# EUROPEAN PATENT SPECIFICATION

(11) **EP 0 569 448 B1**
(45) Date of publication and mention of the grant of the patent: **18.06.1997**
(21) Application number: 92904055.8
(22) Date of filing: 28.01.1992
(51) Int. Cl.: C21C 5/30

(54) **A METHOD OF MANUFACTURING STAINLESS STEEL**
VERFAHREN ZUR HERSTELLUNG ROSTFREIEN STAHLS
PROCEDE DE FABRICATION D'ACIER INOXYDABLE

(30) Priority: 31.01.1991 SE 9100294
(43) Date of publication of application: 18.11.1993
(73) Proprietor: AGA AKTIEBOLAG, 181 81 Lidingö (SE)
(72) Inventor: BRUNNER, Mikael, S-183 30 Täby (SE)
(74) Representative: Wiedemann, Bernd
(86) International application number: SE9200053
(87) International publication number: WO9213975

(56) References cited:
- EP-A- 0 331 751
- SE-B- 424 448
- SE-B- 435 936

## Description

The present invention relates to a method of producing stainless steel by treating a raw high-carbon steel with gaseous mixtures consisting of oxygen and inert gas with decreasing oxygen to inert gas ratios, thereby lowering the carbon content of the steel in a first stage to a value of 0,2-0,1 and thereafter in a second stage to the desired end carbon content.

From SE-A-435936 it is known to refine steel containing chromium to provide a carbon content less than 0.03 percent by blowing gaseous oxygen onto or into the steel melt in a vessel and in which a stirring action is exerted by blowing in inert gas. In this method a first refining step is effected using gaseous oxygen at atmospheric pressure until the carbon content has dropped to from 0.2 to 0.4 percent and a second refining step is effected in said vessel by continuing the agitation in the melt by inert gas but with interruption of the supply of gaseous oxygen. Thereby the pressure above the melting bath is continuously reduced to or below 10 torr.

From Choulet, R J et al, Canadian Metallurgical Quarterly, vol 10, 1971, No 2, p 129-136 it is known to produce stainless steel by processing high-carbon raw steel with a mixture of oxygen gas and inert gas. During the decarburizing stage of the process, gaseous mixtures are blown into the melt and the ratio of oxygen gas to inert gas is changed progressively from an oxygen-rich mixture to an oxygen-lean mixture, as the carbon content of the raw steel diminishes. The method is known under the designation AOD, Argon Oxygen Decarburization.

From the last mentioned reference it is further known that continueouly changed oxygen/argon proportions for minimum argon usage can be approximated by two or more stepwise changes in gas ratios.

Such a process can be begun with a gaseous mixture that contains four parts of oxygen gas and one part of inert gas, or a gaseous mixture of 4/1. The carbon content of the raw steel at the beginning of the process is between 1 and 1.5%. When the carbon content of the raw steel has fallen to about 0.8%, the oxygen gas/inert gas ratio is changed to 3/1, and then successively to 1/1 and finally to 1/3 at the end of the blow, when the carbon content of the steel has fallen to beneath 0.2%. This mixture ratio is then maintained until decarburization is complete, at which stage the carbon content should have fallen to 0.04%.

In addition to carbon, some chromium is also oxidized during the blowing process. This oxidation of chromium represents a disadvantage, since chromium shall be recovered by reduction of chromium oxide with silicon. Silicon is an expensive alloy. The efficiency of the process can be measured by the quantity of silicon consumed.

The change in the mixing ratio between oxygen gas and inert gas is intended to avoid oxidation of chromium to the greatest possible extent. This can only be achieved partially under operating conditions, and consequently some chromium is always oxidized, resulting in the consumption of silicon for the reduction of chromium oxide.

The differing mixture ratios of oxygen gas to inert gas cause difficulties and time losses during the decarburizing process. For example, it is necessary to interrupt the process and to check the carbon content of the molten bath in order, to ascertain the correct mixture ratio to be used. Conventional interruptions and sampling processes prolong the process time, increase sampling costs and analysis costs and also increase the heat losses that occur during the process. It has been proposed that endeavors are made to calculate the carbon content of the bath with the use of expensive analysis instruments, without interrupting the process for the purpose of taking samples and sample analysis. Even though these endeavors achieve the result desired, the instrumentation required in this regard complicates the process of manufacture and therewith also results in higher costs for instrument investment and for maintenance.

An object of the present invention is to provide a decarburization process for the manufacture of stainless steel in which oxygen gas and inert gas are used without changing the mixture ratio as a function of the carbon content. The extent to which chromium is oxidized is equally as low as the level of chromium oxidation that occurs in the conventional method, in which differing oxygen gas/inert gas mixture ratios are applied.

This object is achieved by a process as defined in claim 1. Preferred embodiments are defined in the depending claims.

According to the present invention, the decarburizing process is effected with solely one mixture ratio, for example a mixture ratio of four parts of oxygen gas and one part of inert gas, 4/1. This mixture ratio is maintained until the carbon content has fallen to low values, for example a value of 0.2%. Thus, the same mixture ratio is used while decarburizing from 1.5 to 0.2%. During this period, considerable quantities of inert gas are blown into the bath in short periods of time. These periodic injections of inert gas into the bath result generally in the same decarburizing process as that achieved with the changed mixture ratios applied in accordance with conventional techniques.

The short periods of inert gas injection can take place at a predetermined periodicity, for example a two-minute inert-gas injection at five minute intervals. The inert-gas blowing or injection periods are predetermined and are independent of the carbon content of the bath, and consequently the process can be continued without needing to interrupt the process for the purpose of taking samples and analyzing said samples. When proceeding in accordance with the invention, the extent to which chromium is oxidized becomes smaller rather than greater, and the process time becomes shorter and productivity therefore higher.

The difference between the present invention and the conventional method is considerable and also fundamental. According to the conventional method, the chromium is safeguarded against oxidation by the changed mixture ratios. Oxidation of the chromium is restrained successively by mixtures which are progressively leaner in oxygen, while oxidation of the carbon is promoted at the same time. Thus, according to the conventional method, the purpose of the inert gas is to promote the oxidation of carbon as compared with the oxidation of the chromium.

The present invention is based on the use of a totally different mechanism. The periodically repeated injections of inert gas into the bath result in a chemical reaction between the carbon that is present in the bath and the oxygen that is bound to chromium in the form of chromium oxide. The chromium oxide is thus reduced with carbon during the injection of inert gas into the melt.

This would explain the surprising fact that the process can be carried out without changing the oxygen gas/nitrogen gas ratio in the gaseous mixture blown into the bath. It should be mentioned, however, that this explanation need not constitute a scientific truth. Another explanation may be that the conventional method which utilizes varying ratios of oxygen gas/inert gas is quite simply unnecessary and can therefore be omitted without serious detriment.

In practice, however, the most significant difference between the inventive method and the conventional method is found in the greater efficiency that is achieved when practicing the present invention, especially since the process of changing the mixture ratio between oxygen and inert gas at specific carbon contents, involving stopping the process, sampling, and prolonged waiting times, cannot always be carried out with satisfactory accuracy, despite the time taken and the investment made in expensive measuring instruments.

### Example 1

A raw steel had the following analysis (%):

| C | Si | Mn | Cr | Ni |
|---|---|---|---|---|
| 1.21 | 0.31 | 1.13 | 17.21 | 8.95 |

The molten raw steel was treated in a 5-tonne converter, by blowing oxygen gas and nitrogen gas into the bath. The treatment process was carried out in three stages: A first stage using four parts of oxygen and one part of nitrogen gas and then one part of oxygen and one part of nitrogen gas, and finally with a mixture containing one part of oxygen and three parts of argon. The switching points between the different stages was based on carbon concentrations of 0.53% C and 0.18% C. The final carbon content was 0.041%.

| Time taken: | |
|---|---|
| Stage 1 | 32 min. |
| Stage 2 | 9 min. |
| Stage 3 | 12 min. |
| Sample 1 | 5 min. |
| Sample 2 | 4 min. |
| Sample 3 | 5 min. |
| Reduction, including slagging-off | 17 min. |
| Adjustment | 11 min. |
| Tapping | 3 min. |
| Total | 98 min. |
| | |

| Material consumption: | |
|---|---|
| Oxygen gas | 29.04 Nm³/t |
| Nitrogen gas | 18.10 " |
| Argon | 10.07 " |
| Silicon | 20.32 kg/t |
| Lime | 70.28 " |

### Example 2

A raw steel was treated in a 5-tonne converter. The steel had the following analysis (%):

| C | Si | Mn | Cr | Ni |
|---|---|---|---|---|
| 1.24 | 0.37 | 1.32 | 18.3 | 9.01 |

The treatment process was carried out in accordance with the present invention. A gas mixture consisting of four parts of oxygen gas and one part of nitrogen gas was first blown (injected) into the molten bath. 7 minutes after commencing the blow, nitrogen gas was blown into the bath over a blow-period of 30 seconds, the flow of nitrogen gas reaching to 0.81 Nm³/min., tonne. The injection of four parts of oxygen gas and one part of nitrogen into the bath was then recommenced. After a total blowing time of 12 minutes, nitrogen gas was injected or blown into the bath over a blow-period of 30 seconds, reaching a flow level of 0.81 Nm³/min., tonne. The nitrogen-gas injection period was then repeated at 5-minute intervals. A total of six nitrogen blowing periods was applied. A carbon sample was taken after a blowing time of 38 minutes, and was found to contain 0.17% carbon. Thereafter, only argon was blown into the bath, over a blow-period of 7 minutes, the argon flow reaching to 0.73 Nm³/min., tonne. The final carbon content was 0.039%.

| Time taken: | |
|---|---|
| Stage 1, including nitrogen blows | 38 min. |
| Stage 2 | 12 min. |
| Sample 1 | 5 min. |
| Reduction, including slagging-off | 18 min. |
| Adjustment | 11 min. |
| Tapping | 4 min. |
| Total | 88 min. |
| | |

| Material consumption: | |
|---|---|
| Oxygen gas | 27.22 Nm³/t |
| Nitrogen gas | 17.10 " |
| Argon | 11.02 " |
| Silicon | 18.02 kg/t |
| Lime | 62.31 " |

It will be seen from the two examples that a time saving of 10 minutes was achieved with the inventive method, corresponding to a productivity gain of about 10%. The inventive method also results in a lower silicon consumption, whereas the remaining consumption values are generally the same.

Thus, it will be seen from the examples that the inventive method results in an increase in productivity and also in a lower consumption of materials.

When reference is made to an oxygen-rich gas in the description and Claims of this document, there is meant, in accordance with the present invention, a gaseous mixture which consists of at least 15 percent by volume oxygen, with the remainder consisting of an inert gas, for instance nitrogen or argon. The gaseous mixture will preferably contain at least 70% oxygen. A preferred oxygen range is 75-90%. By inert gas is meant a gaseous mixture containing at least 70 percent by volume of an inert gas, e.g. nitrogen. According to the present definition, air can also be considered as an inert gas. The present inert gas contains at least 90%, particularly at least 99% inert gas, for instance argon or nitrogen.

## Claims

1. A method of producing stainless steel by treating a raw high-carbon steel with a gaseous mixture of oxygen and inert gas,thereby lowering the carbon content of the steel in a first stage to a value of 0,2-0,1 percent by weight, and thereafter in a second stage to the desired end carbon content, **characterized** by:
- treating said steel alternately with an oxygen rich gas mixture containing at least 15 % by volume oxygen and with an inert gas mixture containing at least 70 % by volume inert gas during the whole period of said first stage, the concentration of oxygen in the oxygen rich gas mixture and the concentration of inert gas in the inert gas mixture being maintained constant,
- interrupting then the supply of said oxygen rich gas and blowing an inert gas mixture containing at least 70 % by volume inert gas into the bath during the whole period of said second stage.

2. A method according to Claim 1, **characterized** by treating the steel bath with inert gas in the first treatment stage over a period of time which constitutes 50-5% of the time over which the steel bath is treated with the oxygen-rich gas.

3. A method according to Claim 1 or 2, **characterized** by repeating the treatment with inert gas in the first stage at constant time intervals.

4. A method according to one or more of Claims 1-3,
**characterized** by effecting inert-gas treatment in the first stage over time periods of mutually equal durations.

5. A method according to one or more of Claims 1-4,
**characterized** in that the oxygen content is at least 70%, preferably 75-90%.

6. A method according to one or more of Claims 1-5,
**characterized** in that the inert gas used in the first stage is nitrogen.

7. A method according to one or more of Claims 1-5,
**characterized** in that the inert gas used in the first stage is argon.

8. A method according to one or more of Claims 1-5,
**characterized** in that the inert gas used in the first stage is air.

## Patentansprüche

1. Verfahren zum Herstellen von Edelstahl durch Behandeln eines kohlenstoffreichen Rohstahls mit einer Gasmischung von Sauerstoff und Inertgas, wodurch der Kohlenstoffgehalt des Stahls in einer ersten Stufe auf einen Wert von 0,2 bis 0,1 Gew.-% und danach in einer zweiten Stufe auf den gewünschten Kohlenstoffendgehalt vermindert wird, gekennzeichnet durch:
- abwechselndes Behandeln des Stahls mit einer sauerstoffreichen, wenigstens 15 Vol.-% Sauerstoff enthaltenden Gasmischung und mit einer wenigstens 70 Vol.-% Inertgas enthaltenden Inertgasmischung während des gesamten Zeitraums der ersten Stufe, wobei die Konzentration des Sauerstoffs in der sauerstoffreichen Gasmischung und die Konzentration des Inertgases in der Inertgasmischung konstant gehalten werden,
- Unterbrechen der Zufuhr des sauerstoffreichen Gases und Einblasen einer wenigstens 70 Vol-% Inertgas enthaltenden Gasmischung in das Bad während des gesamten Zeitraums der zweiten Stufe.

2. Verfahren nach Anspruch 1, gekennzeichnet durch Behandeln des Stahlbads mit Inertgas in der ersten Behandlungsstufe über einen Zeitraum, der 50 bis 5 % der Zeit ausmacht, in der das Stahlbad mit dem sauerstoffreichen Gas behandelt wird.

3. Verfahren nach Anspruch 1 oder 2, gekennzeichnet durch Wiederholen der Behandlung mit Inertgas in der ersten Stufe in konstanten Zeitintervallen.

4. Verfahren nach einem oder mehreren der Ansprüche 1 bis 3, gekennzeichnet durch Ausführen der Inertgasbehandlung in der ersten Stufe über Zeitabschnitte von gegenseitig gleicher Dauer.

5. Verfahren nach einem oder mehreren der Ansprüche 1 bis 4, dadurch gekennzeichnet, daß der Sauerstoffgehalt wenigstens 70, bevorzugt 75 bis 90 % beträgt.

6. Verfahren nach einem oder mehreren der Ansprüche 1 bis 5, dadurch gekennzeichnet, daß das in der ersten Stufe verwendete Inertgas Stickstoff ist.

7. Verfahren nach einem oder mehreren der Ansprüche 1 bis 5, dadurch gekennzeichnet, daß das in der ersten Stufe verwendete Inertgas Argon ist.

8. Verfahren nach einem oder mehreren der Ansprüche 1 bis 5, dadurch gekennzeichnet, daß das in der ersten Stufe verwendete Inertgas Luft ist.

## Revendications

1. Un procédé de production d'acier inoxydable par traitement d'un acier brut d'une haute teneur en carbone avec un mélange gazeux d'oxygène et de gaz inerte, de manière à abaisser la teneur en carbone de l'acier dans un premier stade à une valeur de 0,2-0,1 pour cent en poids, et ensuite dans un second stade à la teneur finale désirée en carbone, caractérisé en ce que :
- on traite l'acier alternativement avec un mélange de gaz riche en oxygène contenant au moins 15 % en volume d'oxygène et avec un mélange de gaz inerte contenant au moins 70 % en volume de gaz inerte durant la période entière du premier stade, la concentration d'oxygène dans le mélange de gaz riche en oxygène et la concentration de gaz inerte dans le mélange de gaz inerte étant maintenues constantes,
- on interrompt l'alimentation en gaz riche en oxygène et on injecte dans le bain un mélange de gaz inerte contenant au moins 70 % en volume de gaz inerte durant la période entière du second stade.

2. Un procédé selon la revendication 1, caractérisé en ce qu'on traite le bain d'acier avec un gaz inerte dans le premier stade de traitement pendant un laps de temps qui constitue de 50 à 5 % du temps pendant lequel le bain d'acier est traité avec le gaz riche en oxygène.

3. Un procédé selon la revendication 1 ou 2, caractérisé en ce qu'on répète le traitement avec un gaz inerte dans le premier stade à des intervalles de temps constants.

4. Un procédé selon une ou plusieurs des revendications 1-3, caractérisé en ce qu'on effectue le traitement avec un gaz inerte dans le premier stade pendant des laps de temps ayant des durées mutuellement égales.

5. Un procédé selon une ou plusieurs des revendications 1-4, caractérisé en ce que la teneur en oxygène est d'au moins 70 %, de préférence de 75 à 90 %.

6. Un procédé selon une ou plusieurs des revendications 1-5, caractérisé en ce que le gaz inerte utilisé dans le premier stade est de l'azote.

7. Un procédé selon une ou plusieurs des revendications 1-5, caractérisé en ce que le gaz inerte utilisé dans le premier stade est de l'argon.

8. Un procédé selon une ou plusieurs des revendications 1-5, caractérisé en ce que le gaz inerte utilisé dans le premier stade est de l'air.
